



US008951644B2

(12) **United States Patent**  
**Burns et al.**

(10) **Patent No.:** **US 8,951,644 B2**  
(45) **Date of Patent:** **Feb. 10, 2015**

(54) **THERMALLY PROTECTIVE MULTIPHASE PRECIPITANT COATING**

(75) Inventors: **Andrew J. Burns**, Orlando, FL (US); **Anand A. Kulkarni**, Oviedo, FL (US)

(73) Assignee: **Siemens Energy, Inc.**, Orlando, FL (US)

(\*) Notice: Subject to any disclaimer, the term of this patent is extended or adjusted under 35 U.S.C. 154(b) by 1811 days.

(21) Appl. No.: **11/950,791**

(22) Filed: **Dec. 5, 2007**

(65) **Prior Publication Data**

US 2013/0230739 A1 Sep. 5, 2013

**Related U.S. Application Data**

(60) Provisional application No. 60/973,560, filed on Sep. 19, 2007, provisional application No. 60/974,558, filed on Sep. 24, 2007, provisional application No. 60/974,561, filed on Sep. 24, 2007, provisional application No. 60/974,564, filed on Sep. 24, 2007.

(51) **Int. Cl.**

**B32B 15/04** (2006.01)  
**B32B 15/20** (2006.01)  
**C23C 28/00** (2006.01)  
**C23C 30/00** (2006.01)

(Continued)

(52) **U.S. Cl.**

CPC ..... **F01D 25/005** (2013.01); **C23C 28/325** (2013.01); **C23C 28/3455** (2013.01); **C23C 28/3215** (2013.01); **C23C 30/00** (2013.01); **C23C 28/345** (2013.01)  
USPC ..... **428/680**; 428/632; 428/633; 428/668; 428/678; 416/241 R

(58) **Field of Classification Search**

CPC .... B32B 15/01; B32B 15/016; B32B 15/017;

B32B 15/04; B32B 15/043; B32B 15/20;

B32B 2311/22; B32B 2311/24; B32B

2603/00; C23C 28/00; C23C 28/021; C23C

28/022; C23C 28/028; C23C 28/3215; C23C

30/00; C23C 30/005; C23C 4/085

USPC ..... 428/623, 627, 630, 631, 632, 633, 668,

428/678, 680

See application file for complete search history.

(56)

**References Cited**

U.S. PATENT DOCUMENTS

4,485,151 A 11/1984 Stecura  
4,503,130 A \* 3/1985 Bosshart et al. ..... 428/632  
(Continued)

FOREIGN PATENT DOCUMENTS

DE 3842301 \* 6/1990  
WO 99/49100 \* 9/1999

OTHER PUBLICATIONS

Machine Translation, Singheiser Lorenz, DE 3842301, Jun. 1990.\*  
(Continued)

*Primary Examiner* — Michael E La Villa

(57) **ABSTRACT**

A thermally protective coating (21), such as may be used over a nickel-based superalloy substrate (24). The protective coating (21) includes a CoNiCrAlY or a NiCoCrAlY material and addition of given amounts of one or more secondary elements. The secondary element(s) facilitate and/or join in one or more precipitation mechanisms ( $\gamma'$ , B2) that retain an aluminum reservoir in the protective coating (21), reducing aluminum diffusion into the substrate (24). This aluminum reservoir maintains a protective alumina scale (38) on the coating (21), thus improving coating life and allowing higher operating temperatures.

**5 Claims, 4 Drawing Sheets**



(51) **Int. Cl.**  
**F01D 5/28** (2006.01)  
**F01D 25/00** (2006.01)

8,039,117 B2 \* 10/2011 Kulkarni et al. .... 428/632  
8,043,717 B2 \* 10/2011 Kulkarni et al. .... 428/632  
2002/0132132 A1 9/2002 Bose et al.  
2003/0054108 A1 3/2003 Beele  
2005/0287296 A1 12/2005 Wadley et al.  
2007/0116980 A1 5/2007 Schmitz et al.  
2008/0032105 A1 \* 2/2008 Taylor ..... 428/215  
2008/0163785 A1 \* 7/2008 Hardwicke et al. .... 106/1.21

(56) **References Cited**

## U.S. PATENT DOCUMENTS

4,615,864 A 10/1986 Dardi et al.  
6,168,874 B1 1/2001 Gupta et al.  
6,207,297 B1 3/2001 Sabol et al.  
6,296,447 B1 10/2001 Rigney et al.  
6,376,015 B1 4/2002 Rickerby  
6,440,496 B1 8/2002 Gupta et al.  
6,555,179 B1 4/2003 Reeves et al.  
6,610,419 B1 8/2003 Stamm  
6,677,064 B1 1/2004 Subramanian  
6,896,488 B2 5/2005 Bruce et al.  
6,924,046 B2 8/2005 Stamm  
7,150,921 B2 12/2006 Nelson et al.  
7,198,462 B2 4/2007 Merrill et al.  
7,244,467 B2 7/2007 Grossman et al.  
7,250,222 B2 7/2007 Halberstadt et al.

## OTHER PUBLICATIONS

A.M. Smyslov, A.A. Bybib, R.R. Nev'Yantseva; "Effect of ion implantation and plasma surface treatment on exploitation properties of heat-resistant Ni alloy"; Database CA [online] Chemical Abstracts Service, Columbus, Ohio US 2007; Retrieved from STN Database accession No. 148:384059 abstract.  
Keith E. Knipling, David C. Dunand, David N. Seidman; "Criteria for developing castable, creep-resistant aluminum-based alloys—A review"; Magazine for Metallurgy, Mar. 2006; vol. 97, No. 3; XP001244723; ISSN: 0044-3093; Munich Germany.

\* cited by examiner

**FIG 1 PRIOR ART****FIG 2**

**FIG 3A PRIOR ART****FIG 3B PRIOR ART****FIG 3C PRIOR ART****FIG 4A****FIG 4B****FIG 4C**



FIG 6



## 1

## THERMALLY PROTECTIVE MULTIPHASE PRECIPITANT COATING

## CROSS REFERENCE TO RELATED APPLICATIONS

This application claims the benefit of four U.S. provisional patent applications: 60/973,560, filed Sep. 19, 2007; 60/974,558, filed Sep. 24, 2007; 60/974,561, filed Sep. 24, 2007; and 60/974,564, filed Sep. 24, 2007. These provisional applications are incorporated by reference herein in their entirety.

## FIELD OF THE INVENTION

The invention relates generally to thermally protective coatings for metal structures.

## BACKGROUND OF THE INVENTION

Gas turbine components are subjected to rigorous mechanical loading, thermal stress, oxidation, corrosion, and abrasion. Hot gas path components of such turbines are often made of nickel or cobalt based superalloys optimized for resistance to high temperature creep and thermal fatigue. Protective coatings are applied to increase durability and field performance at high temperatures. MCrAlY (where M represents a transition metal, and Y represents yttrium) is a material commonly used as a protective coating, especially as a bond coat for an overlying ceramic insulation as part of a thermal barrier coating (TBC) system. Such bond coats prevent the substrate from being deteriorated by oxygen, and they act as an intermediary to bridge the difference in the coefficients of thermal expansion (CTE) between the ceramic and metallic materials, thereby reducing stress levels.

MCrAlY materials have been optimized for thermal and chemical compatibility with the superalloys along with oxidation and corrosion resistance. In gas turbine components, the M in MCrAlY is normally nickel (Ni) and/or cobalt (Co). Nickel-based alloys provide superior oxidation resistance, and cobalt-based alloys provide superior corrosion resistance. The chromium (Cr) provides hot corrosion resistance, and aluminum (Al) aids in formation of a stable oxide barrier. Yttrium (Y) enhances adherence of the oxide layer. Elemental additions of cerium, silicon, lanthanum or hafnium to the bond coats are done to improve their performance in terms of the oxidation or thermo-mechanical behavior and ceramic coating adherence. Performance of a TBC often depends on the ability of the underlying MCrAlY bond coating to form a tenacious, protective, aluminum oxide scale that is thermodynamically stable, slow growing, adherent, and that inhibits interactions between the substrate surface and the outside corrosive environment.

## BRIEF DESCRIPTION OF THE DRAWINGS

The invention is explained in the following description in view of the drawings that show:

FIG. 1 is a prior art sectional view of a metal substrate with a bond coat and a thermal barrier coating, illustrating diffusion of aluminum and depletion of a beta phase  $\beta$  from the bond coat.

FIG. 2 is a sectional view of a metal substrate with a bond coat that traps diffusing aluminum within one or more secondary phases, providing an aluminum reservoir that delays aluminum depletion according to an aspect of the invention.

FIG. 3A illustrates a prior art MCrAlY coating on a superalloy substrate.

## 2

FIG. 3B illustrates the coating of FIG. 3A during high temperature operation.

FIG. 3C illustrates the coating of FIG. 3A after total  $\beta$ -phase depletion, marking the end the coating lifespan.

5 FIG. 4A illustrates an MCrAlY coating having first and second layers on a superalloy substrate according to an aspect of the invention.

10 FIG. 4B illustrates the coating of FIG. 4A during high temperature operation illustrating how the first layer traps escaping aluminum in one or more secondary phases, thereby delaying depletion.

FIG. 4C illustrates the coating of FIG. 4A after total  $\beta$ -phase depletion, marking the end the coating lifespan.

15 FIG. 5 is a graph of weight gain over time for various protective coatings, illustrating relative oxidation time and durability.

FIG. 6 is a graph of  $\beta$ -phase depletion times per temperature with a conventional bond coat and with an improved coating system according to the invention.

## DETAILED DESCRIPTION OF THE INVENTION

FIG. 1 shows a known thermal barrier coating system 20 including a bond coat 22 of MCrAlY (such as CoNiCrAlY) 25 adherent to a nickel-based superalloy substrate 24, and a ceramic insulation thermal barrier coating (TBC) 26 adherent to the bond coat. Typically, such a bond coat 22 includes a two-phase region, beta ( $\beta$ ) plus gamma ( $\gamma$ ), in which a matrix  $\gamma$  carries an aluminum rich beta phase  $\beta$ . In one example, an 30 aluminum rich nickel aluminide phase (beta  $\beta$  or NiAl) is carried within a cobalt, nickel, and chromium rich matrix phase (gamma  $\gamma$ ). The matrix  $\gamma$  increases the ductility of the coating, thereby improving thermal fatigue resistance. At 35 high temperatures, diffusion interactions 28, 30 result in depletion of the aluminum, due to formation of an aluminum oxide layer 38 on the top of the bond coat. As the concentration of aluminum decreases, the  $\beta$  phase tends to dissolve. For this reason, the  $\beta$  phase may be described as an aluminum reservoir, and the coating life may be measured in terms of 40 depletion of  $\beta$ . Diffusion interactions of this system in an oxidizing environment form outer and inner  $\beta$  depletion zones 32, 34 as a function of time and temperature. Within the 45 substrate 24 a diffusion zone 36 forms which is termed the interdiffusion zone.

A thermally grown oxide (TGO) layer 38 such as aluminum oxide forms on the outer surface of the bond coat 22 due to exposure of the layer to oxygen at high temperatures. In a TBC system comprising a superalloy substrate, a bond coat, and a ceramic topcoat, this oxide layer, which forms between the ceramic insulation 26 and the bond coat 22, provides insulation from further oxidation, corrosion, and heat. The TGO layer 38 grows during high temperature operation by diffusion 28 of aluminum to the outer surface of the bond coat 22 in the presence of oxygen diffused through the TBC layer 50 26.

55 The formation of the outer  $\beta$  depletion zone 32 is primarily driven by the formation of the oxide layer 38 at the outer surface of the bond coat 22. This depletes the concentration of aluminum in the metal adjacent to the oxide. Thus, outer  $\beta$  depletion is proportional to the growth of the oxide scale. The inner  $\beta$  depletion 30 is a function of  $\beta$ -phase instability in the presence of changing matrix  $\gamma$ -phase compositions in the bond coat 22 caused by substrate/coating interdiffusion. For some superalloy compositions, the inward loss 30 of the  $\beta$  phase to the substrate 24 is more rapid at a given temperature than is the outward loss 28 of the  $\beta$  phase to the TGO 38. Since 60 aluminum lost through inner  $\beta$  phase depletion is not utilized

for TGO **38** growth, it is essentially wasted for the function it was applied to perform, i.e. availability for maintenance of the passive oxide scale **38**. The present inventors have appreciated that any amount of inner  $\beta$  depletion contributes to a debit from the ideal coating oxidation resistance. Thus, it is proposed herein to control aluminum diffusion in the bond coat—particularly the inward diffusion of aluminum atoms into the substrate **24**.

One way to reduce aluminum diffusion is to delay diffusion within the bond coat **22** itself, and/or slow its migration. This can be achieved by certain elemental additions to an MCrAlY bond coat material that modify the beta phase structure, or which catalyze and/or recombine with the diffusing aluminum to precipitate secondary aluminum-rich phases  $\gamma'$  (with about 6 wt % Aluminum (Al)) and B2 (with about 7 wt % Aluminum (Al)) within the bond coat. These secondary phases recapture the aluminum temporarily, thus slowing its migration.

The new element(s) combine with diffusing elements in such a way as to promote and stabilize new aluminum rich phases in the region of the original coating/substrate interface. Thus, inner  $\beta$ -phase dissolution **30** is delayed, leading to prolonged life of the coating system. Creating one or more stable second aluminum-rich phases  $\gamma'$ , B2 requires addition of one or more element(s) that combine with the escaping aluminum in a diffusion interaction to form solid precipitant phases. The additional elements may be selected from strontium (Sr), ruthenium (Ru), lanthanum (La), praseodymium (Pr), neodymium (Nd), promethium (Pm), samarium (Sm), europium (Eu), gadolinium (Gd), terbium (Tb), dysprosium (Dy), holmium (Ho), erbium (Er), thulium (Tm), ytterbium (Yb), tantalum (Ta), rhenium (Re), and combinations thereof. The  $\gamma'$  phase is typically NiAl<sub>3</sub> and the B2 phase is typically complex precipitates (Aluminides of nickel, cobalt, chromium and one of the additional elements from above). These elements are called “seed elements” herein, and an MCrAlY layer modified with them in prescribed amounts is called a “seed layer”. Some examples of these additions are tabulated below, showing their mechanisms of improvement. Certain combinations of such additions have special synergies, as tabulated below. A seed layer **21** will maintain a high aluminum concentration or reservoir in and above the original coating/substrate interface in the form of metal precipitates.

| COMPOSITION                                                                | MECHANISM                                                                                                           |
|----------------------------------------------------------------------------|---------------------------------------------------------------------------------------------------------------------|
| 1. CoNiCrAlY or NiCoAlY with 1-4 wt % praseodymium                         | Forms B2 phase (can be Al rich PrAl <sub>2</sub> or a complex aluminide of Pr/Ni/Co/Cr) and NiAl <sub>3</sub> phase |
| 2. CoNiCrAlY or NiCoAlY with 1-4 wt % samarium                             | Forms B2 phase (can be Al rich SmAl <sub>2</sub> or a complex aluminide of Sm/Ni/Co/Cr) and NiAl <sub>3</sub> phase |
| 3. CoNiCrAlY or NiCoAlY with 1-4 wt % neodymium                            | Forms B2 phase (can be Al rich NdAl <sub>2</sub> or a complex aluminide of Nd/Ni/Co/Cr) and NiAl <sub>3</sub> phase |
| 4. CoNiCrAlY or NiCoAlY with 1-4 wt % neodymium and 0.2-1.0 wt % ruthenium | Forms combinations of Al rich NdAl <sub>2</sub> , NiAl <sub>3</sub> , and RuAl phases                               |
| 5. CoNiCrAlY or NiCoAlY with 2-5 wt % tantalum and 1-3 wt % lanthanum      | Forms TaAl <sub>3</sub> and refines the beta precipitant size                                                       |

Compositions 1-3 above are examples of a seed layer embodiment with additions of 1-4 wt % of one or more lanthanides, especially praseodymium (Pr), neodymium (Nd), promethium (Pm), samarium (Sm), europium (Eu), gadolinium (Gd), terbium (Tb), dysprosium (Dy), holmium (Ho), erbium (Er), thulium (Tm), ytterbium (Yb), lutetium (Lu), and combinations thereof. Composition 5 above

reduces the average beta precipitant microstructure size by reducing the percentage of precipitants in the 7-10 micron range, and increasing their percentage in the 1-7 micron range. This has been found to slow aluminum diffusion.

5 While this finer particle size provides higher surface area for oxidation, it also provides increased precipitant recombination opportunities.

FIG. 2 shows an aspect of the invention in which an MCrAlY bond coat layer **21** is modified with one or more seed elements, forming a seed layer that delays the aluminum migration as described above. One or more secondary aluminum-rich phases  $\gamma'$ , B2 are formed within the seed layer **21** by mechanisms such as listed above.

Another way to reduce aluminum diffusion into the substrate is to apply an MCrAlY seed layer **21** modified with seed elements, and then apply a second layer **22** on the seed layer. The second layer may be a conventional MCrAlY bond coat **22**, or it may be another seed layer composed according to the invention. In either case, aluminum that would diffuse from the second layer **22** into the substrate **24** is delayed and reserved in the first seed layer **21** by one or more of the mechanisms listed above.

FIGS. 3A-3C show stages in the lifespan of a conventional MCrAlY bond coat **22** on a superalloy substrate **24**. A ceramic insulation outer coating is not shown in order to focus on the bond coat. FIG. 3A shows the bond coat **22** prior to use. FIG. 3B shows  $\beta$  phase depletion **28**, **30** in progress during high temperature operation, producing outer and inner oxidation zones **38**, **39**. FIG. 3C shows the bond coat **22** at the end of its lifespan due to total  $\beta$  depletion.

FIGS. 4A-4C show stages in the lifespan of first and second layers **21**, **22** on a superalloy substrate **24**, where the first layer **21** is a seed layer modified according to the invention, and the second layer **22** is a conventional MCrAlY bond coat. A ceramic outer coating may be used, but is not shown in order to focus on the layers **21**, **22**. FIG. 4A shows the layers prior to use. FIG. 4B shows  $\beta$ -phase depletion **28**, **30** in progress in the second layer **22** during high temperature operation. Inwardly diffusing aluminum **30** precipitates into one or more secondary phases  $\gamma'$ , B2 in the seed layer **21**. This mechanism forms an aluminum reservoir and reduces the concentration of free aluminum atoms at the surface of the substrate **24**. Thus, the seed layer **21** reduces the amount of aluminum that is available to diffuse across the coating/substrate boundary, because a portion of the free aluminum is retained in the reservoir created by the secondary phases. A free aluminum concentration gradient is thereby created across the seed layer **21**, with a lowered concentration of free aluminum being available for diffusion at the substrate surface. FIG. 4C shows the layers **21**, **22** at the end of their lifespan due to total  $\beta$ ,  $\gamma'$ , and B2 depletion. The lifespan of FIG. 4C is longer than that of FIG. 3C with equivalent operating conditions, layer **22** compositions, and total thickness.

The first layer **21** may have chemistry similar to that of the second layer **22**, but may incorporate one or more of the above seed elements not found in the second layer. Thus, the first and second layers **21**, **22** may be considered distinct for discussion and illustration purposes. In practice, the first layer **21** may be a subset of the overall thickness of the second layer **22** wherein specific elements have been added and are available for the formation of secondary metal precipitants desired as an aluminum reservoir. One or more seed elements may be added throughout a seed layer or only to a region of the coating that is remote from a surface where it is desired to form a protective alumina layer **38**. For example, an MCrAlY layer with seed elements concentrated adjacent the substrate may be achieved by means of layered deposition using atmo-

spheric/low pressure/vacuum plasma or high velocity oxy-fuel spraying. The first layer thickness may be 50-200 micrometers, with a preferred range of 75-125 micrometers. In a two-layer system, the combined thickness of the two layers may be in the range of 125 to 325 micrometers.

Multiple layers with the new elemental additions may be used. The presence of multiple seed layers forms multiple precipitated aluminum phases as diffusion progresses. When multiple seed layers are used, they may have the same or different compositions from each other.

MCrAlY bond coat compositions can be modified to improve oxidation and corrosion resistance and thermo-mechanical properties by additional alloying elements or by an oxide dispersion in the matrix. Additions of hafnium (Hf), platinum (Pt), titanium (Ti), tungsten (W), and/or tantalum (Ta) offer oxidation resistance. Addition of rhenium (Re) improves isothermal or cyclic oxidation resistance and thermal cycle fatigue. One or more of these elements may be incorporated in a first and/or second layer of the present invention to provide these improvements.

FIG. 5 compares results of prior bond coating options and the present invention, both as a single layer and with two layers, by respective weight gained due to oxidation over time for various protective coatings. A coating life is proportional to the time required for a given weight gain. All of the illustrated samples undergo a change in slope after some passage of time that indicates  $\beta$ -phase depletion. Upon complete  $\beta$  phase depletion, the oxidation of the system behaves like a bare superalloy; hence the breakaway slope is similar for all systems 50, 52, 54, 56, 58, 59. Since there is no  $\beta$ -phase in superalloys, the weight gain starts earlier with a bare superalloy 50 than with coated systems 52, 54, 56, 58, 59. With an MCrAlY coating 52, first the  $\beta$  depletion occurs in the coating, then after total depletion, the system oxidizes at the same rate as substrate. Modifying the MCrAlY bond coat chemistry 54 with platinum, hafnium, tantalum, and/or tungsten, or modifying it 56 with rhenium, increases its oxidation resistance (total  $\beta$ -phase depletion times). Further improvement is shown with addition 58 of a seed layer under an MCrAlY bond coat as proposed herein. Even better improvement is shown by modifying 59 the bond coat itself with seed layer additions listed herein, making it serve singly as both the bond coat and seed layer.

For example, the bond coat and/or the seed layer(s) may be composed of MCrAlY with 8-12 wt % aluminum and 1-2 wt % rhenium, and the seed layer(s) or the single bond/seed layer may further comprise one or more of the listed seed layer additions.

A seed layer may be 50 to 200 micrometers thick with a preferred range of 75-125 micrometers. Each elemental addition results in a given composition of precipitants and mechanism of performance improvement. The listed combination of 2-5 wt % tantalum and 1-3 wt % lanthanum has a dual mechanism—it both reduces the original  $\beta$  phase grain size, and produces a Ta-rich secondary  $\beta$  phase.

FIG. 6 shows general performance benefits of the present coating system compared to conventional bond coat systems. The improvement is expressed as an increased temperature and/or time at temperature. The present system exceeds the temperature limits of conventional TBC systems, thus substantially improving the performance of gas turbines incorporating such coatings.

The conventional bond coat and/or the modified layer(s) may be deposited by known methods such as air plasma or vacuum plasma/low pressure plasma, wire-arc, flame combustion, high velocity oxy-fuel or a cold spray process, depending on the operational requirements. Also, any known

method of forming powders for use in bond coat applications may be used. For example, not to be limiting, a bond coat powder may be prepared by gas atomization of the components to obtain relatively uniform chemistry of the powder particles, which then are deposited or otherwise applied onto a substrate.

Embodiments of the present invention may include components for turbines, such as gas turbine engines, as well as for any other device having a need for a component comprising a thermal barrier system having an advanced bond coat effective to provide increased protection and durability as described herein.

The present invention provides metallic coatings with elemental additions that form secondary and possibly tertiary and quaternary aluminum-rich phase precipitation events. The result of these precipitation events keeps an aluminum reservoir between the oxidizing outer surface of the coating and the substrate rather than allowing the aluminum to diffuse into the substrate base metal, and become unusable for passive oxide growth. This results in superior oxidation resistance and longer life at high temperatures.

While various embodiments of the present invention have been shown and described herein, it will be obvious that such embodiments are provided by way of example only. Numerous variations, changes and substitutions may be made without departing from the invention herein. Accordingly, it is intended that the invention be limited only by the spirit and scope of the appended claims.

30 The invention claimed is:

1. A protective metal coating for a nickel-based superalloy substrate, the protective coating comprising:  
a first layer comprising a CoNiCrAlY or a NiCoCrAlY material on a surface of the substrate;  
an addition to the first layer material of a seed element in an amount of 1-4 wt % selected from the set consisting of praseodymium (Pr), neodymium (Nd), promethium (Pm), samarium (Sm), europium (Eu), gadolinium (Gd), terbium (Tb), dysprosium (Dy), holmium (Ho), erbium, (Er), thulium (Tm), ytterbium (Yb), lutetium (Lu), and combinations thereof; and  
a second layer comprising a CoNiCrAlY or a NiCoCrAlY material on a first layer;  
whereby the first layer forms multiphase precipitant aluminum compounds in combination with aluminum diffusing from the second layer material above a given operating temperature, delaying the diffusing aluminum in reaching the substrate, and forming an aluminum reservoir in the first layer that supports aluminum diffusion through the second layer to an outer surface thereof over an extended period of time;  
wherein the second layer comprises 8-12 wt % aluminum and further comprises 1-2 wt % rhenium.

2. The protective metal coating of claim 1, wherein the 55 second layer further comprises at least one elemental addition selected from the set consisting of hafnium (Hf), platinum (Pt), titanium (Ti), tungsten (W), and/or tantalum (Ta).

3. A protective coating for a nickel-based superalloy substrate, the protective coating comprising:  
a seed layer comprising a CoNiCrAlY or a NiCoCrAlY material on a surface of the substrate; and  
elemental additions to the seed layer material of 1-4 wt % neodymium and 0.2-1.0 wt % ruthenium;  
a second layer comprising a CoNiCrAlY or a NiCoCrAlY material on the seed layer;  
whereby the seed layer forms multiphase precipitant aluminum compounds above a given operating tempera-

ture, including  $\text{NiAl}_3$ ,  $\text{NdAl}_2$ , and  $\text{RuAl}$ , which delay aluminum diffusion from the second layer material into the substrate.

- 4.** A protective coating for a nickel-based superalloy substrate, the protective coating comprising:
- a seed layer comprising a  $\text{CoNiCrAlY}$  or a  $\text{NiCoCrAlY}$  material on a surface of the substrate, and
  - elemental additions to the seed layer material of 2-5 wt % tantalum and 1-3 wt % lanthanum;
- whereby the seed layer forms  $\text{TaAl}_3$  above a given operating temperature, which delays aluminum diffusion from the seed layer material into the substrate.
- 5.** The protective coating of claim 4, further comprising a ceramic thermal barrier coating on the seed layer.

\* \* \* \* \*

15